

## UNITED STATES PATENT OFFICE.

SAMUEL E. SHEPPARD, OF ROCHESTER, NEW YORK, ASSIGNOR TO EASTMAN KODAK COMPANY, OF ROCHESTER, NEW YORK, A CORPORATION OF NEW YORK.

PHOTOGRAPHIC LIGHT-SENSITIVE MATERIAL CONTAINING SELENIUM AND PROCESS OF MAKING THE SAME.

No Drawing. Original application filed June 6, 1924, Serial No. 718,411. Divided and this application filed January 21, 1926. Serial No. 82,847.

This application is a division of my prior Patent Number 1,574,944, dated March 2, 1926, granted on application No. 718,411, filed June 6, 1924 for photographic light sensitive materials and processes of making the same.

This invention relates to the art of photographic materials.

One object of the invention is to provide photographic emulsions, especially developing-out ones, having new or improved properties because of the use or presence therein of materials, the sensitizing properties of which I have discovered. Still another object of my invention is to provide processes in which such materials are used to improve photographic emulsions, especially developing-out ones, as regards light-sensitivity, by which term I include their ability to give the earliest visible impression or image with the minimum exposure or their ability to give density after a given exposure or both, the usual photographic fluid treatments being used in preparing such impression or image or density.

A further object of the invention is to provide colloid products, such for instance as gelatins, the usefulness of which for forming light sensitive photographic emulsions, especially developing-out emulsions, is greatly increased and controlled by my said sensitizing materials incorporated therewith. Another object of the invention is to provide processes for preparing said colloid products or intermediates.

Other objects are,—to increase the sensitivity of photographic emulsions, especially developing-out emulsions, while wholly or partially dispensing with expensive or long and uncertain so-called ripening methods; to enable the use of a type of gelatin having desirable physical qualities in making such a photographic emulsion of greater light-sensitivity than that normally obtainable with said gelatin; to obtain more stable emulsions through the purity of the ingredients; to increase the light-sensitivity of photographic emulsions, particularly developing-out ones, the grain characteristics of which have already been determined; to increase the general light-sensitivity of such photographic emulsions

throughout the spectral ranges to which they are normally sensitive; to make such photographic emulsions of standard light-sensitivity characteristics with gelatins which normally do not produce emulsions having such characteristics; to make, as intermediates in the manufacture of photographic emulsions, gelatins of standard light-sensitivity giving power out of gelatins which do not normally have the power of giving such standard sensitivity to emulsions, such as developing-out ones, made from them. Further objects will hereinafter appear.

I have found that a series of chemical compounds produce remarkable light-sensitizing effects upon photographic emulsions, especially developing-out ones when incorporated therein. Broadly speaking each compound of these series contains a divalent selenium atom which is joined by a double bond to a single metalloid atom (not one bond to one atom, and the other bond to a different atom) to which at least another group of atoms is attached. Generally it is desirable that the last mentioned group of atoms be such that it induces in the compound a chemical affinity for silver halids,—for instance the compound may combine to an appreciable extent with silver halid to form a soluble complex salt, when said atomic group is present. Moreover, the metalloid atom to which the atom of selenium is joined by a double bond is in many instances, but not necessarily, a carbon atom.

For some of the preferred examples of my invention, I select from the above series the following subseries selenocarbamids. As the corresponding carbimids are likewise usable in preferred examples of my invention and are readily changed into said carbamids, especially for instance in emulsions of the alkaline or ammonia type, it will be understood that the corresponding carbimids are included hereinafter when said carbamids are claimed. These subseries of carbamids and carbimids include many compounds containing one or more substituent radicals, such as alkyl, aryl, acyl, alkyl-oxy, aryl-oxy, etc., groups. Examples are allyl isoselenocyanate, allyl selenourea. Not only can each compound of my series of light-sensitizers

be used alone to improve an emulsion (or colloid for an emulsion) but two or more of such compounds may be used together to obtain their mutual or cumulative effects.

5 It is a common characteristic of the compounds which I use, that said double bonded selenium atom is chemically held in the molecule with intermediate firmness. Such atom does not react on silver halids as readily as 10 the sulfur atom in sodium sulfide for instance, but it separates out more readily than the sulfur atom in ethyl mercaptan for example. Consequently said double bonded sulfur-group atoms in my compounds correspond roughly in the firmness with which 15 they are held to the firmness with which the sulfur atoms are held in the so-called potential mercaptans, although there is, of course, some range of difference in the firmness with 20 which said double-bonded atoms are held in the different compounds of my series. The sensitiveness of the grains of silver halid in emulsions has been shown to correspond to the presence in said grains of nuclei of un- 25 stated chemical composition. I, therefore, attribute the sensitizing action of my compounds to their forming in the emulsion grains small, mostly ultramicroscopic, nuclei which include silver combined with selenium. 30 The intermediate firmness with which said double-bonded atoms are held in my compounds facilitates this scattered formation or reaction without reacting on the whole of each grain. Since this deduction is not in- 35 dispensable to the practical using of my invention, I do not wish to be limited to it except as defined in the claims.

I have also found that the proportions in 40 which my compounds are incorporated in the emulsions (or in the colloids for the emulsions) are important. If used in too high concentrations, they cause fog, and sometimes reversal. The largest proportions which can be effectively used vary somewhat with the particular sensitizing compound or compounds which are used, with the proportion of gelatin to silver halid in the emulsion, with the type of emulsion as regards grain size characteristics and alkalinity, with the 45 amount of natural sensitizer originating in the gelatin when the latter is manufactured, with the particular silver halid or halids employed, the standard as regards fog which is set by the emulsion maker, etc. This maximum proportion is in any specific case easily found, being about as readily determined by routine test as, for example, the proportion of sulfur permissible in steel for a particular purpose. It is, however, always surprisingly 50 small. In general with gelatino-silver-halid developing-out emulsions, it should be less than about 10 grains of active sensitizing compound, in 130 pounds of emulsion (the latter being computed as the weight of its 55 non-aqueous ingredients in the dry state);

or less than about 10 grains in 100 pounds of gelatin (computed as dry gelatin), when it is added to the gelatin before the latter is used in making the emulsion. A quantity which causes immediate fogging tendency 60 should not be used,—that is, a quantity which causes more than the tolerated fog allowed in the particular type of emulsion in the trade after the customarily allowed period of storage. I have found 2 to 3 grains of sensitizing compound, to 100 pounds of gelatin (computed as dry) or 130 pounds of emulsion (computed as dry) is within the useful limits and generally excellent,—say 65 for instance with alkaline developing-out gelatino-silver-halid emulsions. Of course, smaller amounts of sensitizers are employed when less sensitizing effects are desired; but it is important not to exceed the upper limits 75 as stated above.

Because only very minute quantities of my sensitizing compounds are used, (often less than one three hundred thousandth of the weight of emulsion) the addition of them 80 does not appreciably dilute the emulsion or emulsion-forming colloid; nor does it affect their physical properties. Consequently the use of my compounds provides a novel, dependable, and independent way for controlling the properties of photographic emulsions in addition to the customary expedients 85 hitherto available. Gelatins, for instance, can be selected for their physical properties, such as setting ability, melting point and viscosity, without regard to whether they 90 can be made into sufficiently light-sensitive emulsions, and any deficiency in sensitizing power can be made up by incorporating a little quantity of one or more of my independent compounds. Nor are the grain-size 95 characteristics affected by such additions of my compounds, they being independently controlled by the emulsion maker. In other words, I can establish a ratio of sensitizing 100 compounds to silver halid in the emulsions which is independent of the ratio of gelatin to silver halid. Still differently stated, the sensitizing compounds can be added without 105 adding any colloid, such as gelatin, and are 110 therefore, independent thereof.

My sensitizing compounds act as so-called "chemical" sensitizers instead of as "optical" sensitizers. In other words, they increase the "general" sensitiveness of photographic 115 emulsions, notably developing-out ones, in which they are incorporated,—that is to light of substantially the same wave lengths as those to which the emulsion would be sensitive without the incorporation of my compounds; instead of merely increasing the sensitiveness to some narrow group of wave lengths. Unlike the effects of dyes, the sensitiveness is increased throughout the normal spectral range of the emulsion instead 120 of at only those spectral points correspond- 125

ing to the spectral absorption of the sensitizing compound. My compounds are effective in increasing the general light-sensitivity of orthochromatic, panchromatic, 5 X-ray, and all special emulsions, as well as the ordinary or non-color-sensitized ones. They can be added without or with sensitizing dyes or before or after them. They do not specifically affect the dye action; but 10 simply increase the general sensitiveness and thus increase the ordinary sensitiveness to blue light to at least as great an extent as to light of a color corresponding to the dye.

My sensitizing compounds may be used in 15 many ways. Broadly they may be incorporated in emulsions or in colloids for emulsions or both. They can also enter the emulsion mixed with other ingredients thereof whether organic or inorganic. They may 20 be added at different stages of emulsion manufacture, even when the latter is otherwise complete ready for coating. Since their action is rapid when incorporated, the coating in such case need be delayed only 25 long enough to mix in the sensitizing compounds. With the grain characteristics, such as size distribution, etc., already determined, and the other physical and photographic properties of the emulsion already 30 taken care of at this stage, I can practically independently increase its light-sensitivity without impairing said other properties by adding one or more of my compounds. The latter are especially effective in emulsions which are, at least slightly, alkaline.

Where different batches of emulsion, especially developing-out emulsions, fall below a required manufacturing standard of light sensitiveness, although they may be otherwise satisfactory, their sensitiveness can 40 readily be brought up to standard by mixing in my sensitizing compounds, the proportion varying with the increase necessary to produce a uniform product. Emulsions 45 having almost no practical light-sensitivity but having enough other desirable qualities can be made usefully light-sensitive by my compounds. Thus the latter are useful in connection with emulsions having good 50 initial light-sensitivity and those having almost no initial sensitiveness. The increase in sensitiveness can be effected in one step by thoroughly stirring all of the sensitizing compound into the emulsion at one time; or 55 it may be incorporated part at a time in successive steps. When making new batches of emulsion from the same materials which have yielded deficient emulsions, correctional quantities of my sensitizing compounds can 60 be premixed with an ingredient, such as gelatin.

The following example illustrates how light-sensitive photographic emulsions of the developing-out type may be prepared and 65 improved by the aid of one or more of my

sensitizing compounds. Of course, my invention is not restricted to this illustration, except as indicated in the claims. The emulsion-forming operations hereinafter described are along the lines of known practice, see for instance "Die Photographie mit Bromsilber Gelatin" by J. M. Eder, published in Halle, Germany in 1903 by Wilhelm Knapp as Part III of Eder's "Ausführliches Handbuch der Photographie." 70 75

The two following solutions are made up, the parts being by weight:

A. 900 parts of silver nitrate in 9,200 parts of water.

B. 690 parts of potassium bromide and 80 50 parts of potassium iodide in 6,100 parts of water along with 300 parts of gelatin.

In mixing B, the halid salts are first dissolved, the water and the gelatin then added to the salt solution. Solution B is then 85 warmed, say to 140° F. or 150° F. for example; and the silver nitrate solution A is gradually added to it with constant stirring. It is preferable to warm solution A before adding it to B, say to 150° F. or 160° F. 90 for instance. When solution A has been thoroughly incorporated in solution B, there are then added 43 parts of strong ammonia previously dissolved in 900 parts of water. The emulsion formed by these operations is allowed to stand for a short time, 95 say 15 minutes to a half hour for example. Then 1050 parts of gelatin are dissolved in it with thorough mixing. The emulsion is next cooled, such as by keeping in a cool 100 space, until it sets to a firm jelly. The latter is broken up, as by shredding for instance, and thoroughly washed to remove soluble salts, such as potassium nitrate and any excess potassium halids. The wash 105 water is, of course, cool enough not to melt the pieces of emulsion jelly. The washed emulsion is next remelted to 100° F. and 1050 parts of water soaked gelatin are thoroughly mixed into it, the temperature 110 then being raised, say between 120° F. and 150° F., for instance, for a short time, say a few minutes. It is then cooled and set. It is an example of the ammonia or alkaline 115 type of developing-out emulsion.

My sensitizing compounds may be usefully incorporated at any stage of the above described process of preparing the emulsion, even being premixed with solutions A or B or with ammonia or with the gelatin, at the 120 initial stages. When the compounds are incorporated in either a partly or wholly prepared emulsion, they are most conveniently handled by dissolving them in a solvent which is inert with respect to the emulsion and simply acts as a vehicle to help in spreading the compounds throughout the emulsion. So long as an even distribution 125 of the compounds throughout the emulsion is effected and the correct proportion of 130

them is added, their particular concentration in the solvent or vehicle is not important. It is good practice to keep the volume of the solution added to the emulsion under 5 2% of the volume of the emulsion; but this is not indispensable. For example, where 1 part of allyl selenourea by weight is to be incorporated into 300,000 parts by weight of the above described emulsion (computed 10 as the weight of its non-aqueous ingredients) the emulsion is melted, the sensitizer dissolved in ethyl alcohol or water or a mixture of them, the volume of said solvent being under approximately 1.5% of the volume 15 of the melted emulsion, and then the solution is thoroughly mixed into the emulsion. When necessary to minimize dilution, the volume of solution can be kept even below a fraction of 1%. I may mention also as 20 very useful potassium selenocyanide.

With its light-sensitiveness increased by my compounds, the emulsion, being melted to the desired flowability, is coated on its support, such as glass, film, paper, etc., in 25 the well known way. It is convenient to control and check the process by coating samples of the emulsion before and after the addition of my sensitizing compounds, the coated specimens being tried out photographically by any well known sensitometric 30 test, or even by comparative camera exposures on the same subject under like conditions. Of course, the usual precautions are observed during the emulsion making 35 and coating processes, such as the use of non-actinic or "safe" light, cleanliness of vessels and air, etc.

The different gelatins sold for photographic emulsion-making may be used in the 40 example given above, hard ones being very useful. The temperatures given are, of course, adjusted if the particular gelatin employed has physical properties, such as melting and setting points, which deviate 45 considerably from the usual ones, such adjustment being a matter of routine control.

Instead, however, of using gelatins which give emulsions of useful but lower sensitiveness even before the addition of my sensitizing material, an almost inert gelatin may be employed,—one which forms an emulsion 50 which produces a developable image, if at all, only after impractically long exposures, and then does not yield an image of desirable 55 density. A gelatin which forms such a practically inert emulsion may be prepared in the way described under the heading "Preparation of ash-free gelatin" in pages 1856 and 1859 of the "Journal of the 60 American Chemical Society", September, 1922, Vol. XLIV, No. 9, being part of an article by Sheppard, Sweet, and Benedict on "Elasticity of purified gelatin jellies as a function of hydrogen-ion concentration." 65 Emulsions of impractically low light-sen-

sitiveness made by the above described process from such prepared gelatin, are transformed by my sensitizing compounds into emulsions which give developable images of excellent density after usefully brief exposures. I have, for example, been able to increase the light-sensitiveness of some such low sensitive emulsions ten or even over 70 twenty times, the exposures for a given subject in the latter case being cut to less than 75 one twentieth of the original one and the image density being made excellent by a corresponding gain. Increases of the same 80 general order of magnitude are made when my sensitizing compounds are added in similar proportions to emulsions which are made from normal photographic gelatins or mixtures of such normal gelatins with said almost inert gelatins, and already have useful, but lower initial sensitiveness. Different 85 percentages of sensitizer produce correspondingly different increases. The increases in developing-out emulsions appear upon the usual developing operations. Customary pyro and metolhydrochinon alkaline 90 developers are suitable for example. An inert emulsion prepared as above described is a very useful medium or standard in which to test the sensitizing properties of different 95 compounds, a sample containing the compound under test being tried out photographically along with a parallel sample of unsensitized emulsion.

Instead of the inert gelatin prepared according to the reference given in the preceding paragraph, I can prepare inert gelatins by treating active photographic gelatins with oxidizing agents. The latter oxidize the sulfur in the sensitizing substituted (allyl) thiocarbamide or corresponding carbimide, which occurs naturally in photographic gelatins, thus converting it to a non-sensitizing compound and leaving the gelatins practically inert. Dilute aqueous 100 solutions of a peroxide, such as sodium peroxide (say from 5 to 10% by weight) is intimately mixed into the gelatin and then washed out when the oxidation has occurred. The inert gelatin referred to in the preceding 105 paragraph can be thus oxidized to make 110 its inertness doubly sure.

When preparing inert gelatin on a considerable scale, it is far preferable to introduce the oxidizing step during the regular 115 manufacturing operations, say the liming and/or deliming treatments. The oxidizing agents should be effective as desensitizers and yet not be present in quantities capable of materially reducing the yield of 120 gelatin or harming its quality, especially its physical properties. Nor should they leave 125 objectionable products from the oxidation reaction. For example, the regular liming solution of the usual gelatin manufacturing process can be saturated with as much cal- 130

cium hypochlorite as will dissolve therein; or it can contain about 5 to 10% of sodium peroxide. Subsequent operations then proceed as usual.

5 My sensitizing compounds may be incorporated into gelatin from which photographic emulsions are to be made. This "strengthened" gelatin then constitutes a valuable "intermediate" in emulsion manufacture. While any good gelatin may be thus treated, that which has been rendered inert by the above described oxidation treatment during liming or deliming is particularly adapted to this strengthening. Emulsions made from the mixture have markedly increased light-sensitiveness as compared with those made from corresponding un-strengthened gelatins. The proportion of sensitizing material is, of course, adjusted to give the desired control of the sensitiveness of emulsions made from the gelatin, the total sensitizing material in the "strengthened" gelatin being thus brought to, or even above, normal.

10 When working on a considerable scale, this activating of gelatin, such, for instance, as said inert gelatin, is one of the most desirable ways of employing my sensitizing compounds. In fact, premixing of one or more of my sensitizers with gelatin is my preferred system. During manufacture of the gelatin, say for instance when the concentrated gelatin solution comes from the evaporator before setting and drying, the sensitizing compound or compounds are added and thoroughly mixed to obtain effectively uniform distribution. For example 2 or 3 grains of any of the hereinabove listed compounds or mixtures of them is carefully mixed with each fraction of gelatin solution containing 100 pounds of gelatin (calculated as dry). The compound is taken up, preferably in as little aqueous-alcohol mixture as is practicable, and then this concentrated solution added to the gelatin solution. In this way undesirable dilution of the latter is avoided.

15 On a large scale, the sensitizing solution may be accurately and continually dosed into a regulated stream of gelatin solution with continuous mixing. Alternatively dried or set gelatin may be allowed to swell in an aqueous solution of the sensitizing compound. The nearly uniform distribution or diffusion of the compound in the gelatin thus effected can be made even more nearly uniform by melting and agitating the swollen gelatin.

20 In the examples given above the steps of treating with ammonia and warming of the emulsion just before its final setting improve the photographic properties of the emulsion, especially when the latter is made from hard gelatins. But one or both of them may be omitted. In other words, my sensi-

tizing compounds act by themselves to increase the light-sensitiveness, whether ripening steps be employed or not, and so can wholly or partially replace them. But I prefer to use them because the effect of either or both of them is to help increase the light-sensitiveness of the emulsion and thus give a stronger initial sensitized condition which is multiplied or increased by using my sensitizing compounds. When using any of the inert gelatins mentioned above in making very sensitive emulsions, these steps can sometimes be shortened and made more certain in effect by reason of the use of my powerful and dependable sensitizing compounds.

25 I have described gelatin emulsions and emphasized the developing-out and alkaline types because at the present time they are the ones which have the widest practical use. Moreover, they form the best medium for testing new sensitizing-compounds. But other organic colloids and mixtures of them with each other or with gelatin, where their nature admits such mixtures, may be used 30 in making light-sensitive emulsions which can be improved by adding my sensitizing material. Albumens, agar-agar, gums, such as gum-arabic, cellulosic derivatives such as collodion are instanced. While I have 35 illustrated the use of my sensitizer in connection with such sensitive substances as silver bromide and silver iodide, other light-sensitive substances can be employed, such as silver chlorid, alone or mixed with one or more of the others.

40 Having thus described my invention, what I claim as new and desire to secure by Letters Patent is:

1. A photographic developing-out emulsion comprising a colloid, particles of photographic silver salt suspended therein, and an added compound therein upon which at least part of the light-sensitiveness of the emulsion depends, said compound containing a divalent selenium atom of the sulfur group directly joined by a double bond to a single metalloid atom to which at least another group of atoms is attached, the proportion of said compound being substantially independent of the proportion of said colloid.

45 2. A photographic developing-out emulsion comprising gelatin, particles of silver halid suspended therein and seleno carbamid upon which at least part of the light-sensitiveness of the emulsion depends.

50 3. A photographic developing-out emulsion comprising gelatin, particles of silver halid suspended therein and allyl selenourea upon which at least part of the light sensitiveness of the emulsion depends.

55 4. A photographic developing-out gelatio-silver-halid emulsion of the alkaline type of relatively high-light-sensitiveness,

comprising a mixture of the constituents of a gelatino-silver-halid emulsion of lower light-sensitiveness and an added sensitizing compound upon which depends the difference between said lower and said high light-sensitiveness, said compound containing a divalent selenium atom directly joined by a double bond to a single metalloid atom to which at least another group of atoms is attached.

5. A photographic developing-out emulsion comprising gelatin, particles of silver halid suspended therein and an added compound therein upon which at least part of the light-sensitiveness of the emulsion depends, said compound containing a divalent selenium atom directly joined by a double bond to a single metalloid atom to which at least another group of atoms is attached, said emulsion being substantially free from sensitizing dye, and the proportion of said compound being substantially independent of the proportion of gelatin.

6. A photographic developing-out emulsion comprising gelatin, particles of photographic silver salt suspended therein and an added compound therein upon which at least part of the light-sensitiveness of the emulsion depends, said compound containing a divalent selenium atom of the sulfur group directly joined by a double bond to a single metalloid atom to which at least another group of atoms is attached, the amount of added compound being less than the order of 10 grains per 130 pounds of emulsion and insufficient to cause immediate fogging tendency.

7. In the process of preparing a developing-out gelatino-silver-halid emulsion, increasing the light-sensitiveness thereof by incorporating with the other constituents thereof a sensitizing compound containing a divalent selenium atom directly joined by a double bond to a single metalloid atom to which at least another group of atoms is attached.

8. In the process of preparing a developing-out gelatino-silver-halid emulsion, increasing the light-sensitiveness thereof by incorporating seleno carbamid with the other constituents thereof.

9. In the process of preparing a developing-out gelatino-silver-halid emulsion, increasing the light-sensitiveness thereof by incorporating allyl selenourea with the other constituents thereof.

10. In the process of preparing a developing-out gelatino-silver-halid emulsion of the alkaline type of relatively high light-sensitiveness, combining constituents of a gelatino-silver-halid emulsion of said type but of lower light-sensitiveness with an independent sensitizing compound, said compound containing a divalent selenium atom

of the sulfur group directly joined by a double bond to a single metalloid atom to which at least another group of atoms is attached.

11. In the process of preparing a developing-out colloid-sensitive-silver-salt emulsion, increasing the light-sensitiveness thereof by incorporating with the other constituents thereof, which are substantially free from sensitizing dye, a sensitizing compound, which is also substantially free from sensitizing dye, said compound containing a divalent selenium atom directly joined by a double bond to a single metalloid atom to which at least another group of atoms is attached.

12. In the process of preparing a developing-out gelatino-silver-halid emulsion, increasing the light-sensitiveness thereof by incorporating with the other constituents thereof a sensitizing compound containing a divalent selenium atom directly joined by a double bond to a single metalloid atom to which at least another group of atoms is attached, the amount of said added compound being less than the order of 10 grains per 130 pounds of emulsion and insufficient to cause immediate fogging tendency.

13. An intermediate for use in making photographic emulsions, comprising an emulsion-forming colloid having incorporated therein a sensitizing compound containing a divalent selenium atom directly joined by a double bond to a single metalloid atom to which at least another group of atoms is attached.

14. An intermediate for use in making photographic emulsions, comprising gelatin having incorporated therein seleno carbamid.

15. An intermediate for use in making photographic emulsions, comprising gelatin having incorporated therein allyl selenourea.

16. An intermediate for use in making photographic emulsions, comprising an emulsion-forming colloid having incorporated therein a sensitizing compound containing a divalent selenium atom directly joined by a double bond to a single metalloid atom to which at least another group of atoms is attached, the amount of said added compound being less than the order of 10 grains in 100 pounds of gelatin.

17. The process of making an intermediate for use in the preparation of photographic emulsions, which comprises incorporating in an emulsion-forming colloid an independent sensitizing compound containing a divalent selenium atom directly joined by a double bond to a single metalloid atom to which at least another group of atoms is attached.

18. The process of making an intermediate for use in the preparation of photo-

graphic emulsions, which comprises incorporating in an emulsion-forming colloid a seleno carbamid.

19. The process of making an intermediate for use in the preparation of photographic emulsions, which comprises incorporating in an emulsion-forming colloid allyl selenourea.

20. The process of making an intermediate for use in the preparation of photographic emulsions, which comprises incorporating in an emulsion-forming colloid an independent sensitizing compound containing a divalent selenium atom directly joined by a double bond to a single metalloid atom to which at least another group of atoms is attached, the amount of said added compound being less than the order of 10 grains per 100 pounds of said colloid (calculated as dry colloid) and being insufficient to cause immediate fogging tendency.

21. The process of making an intermediate for use in the preparation of photographic emulsions, which comprises incorporating in an emulsion-forming colloid a seleno carbamid, the amount of said added compound being less than the order of 10 grains per 100 pounds of said colloid (calculated as dry colloid) and being insufficient to cause immediate fogging tendency.

22. The process of making an intermediate for use in the preparation of photographic emulsions, which comprises incorporating in an emulsion-forming colloid allyl selenourea, the amount of said added compound being less than the order of 10

grains per 100 pounds of said colloid (calculated as dry colloid) and being insufficient to cause immediate fogging tendency. 40

23. The process of making an intermediate for use in the preparation of photographic gelatino-silver-halid emulsions, which comprises substantially freeing gelatin from sensitizing compounds, and incorporating therein a sensitizing compound containing a divalent selenium atom directly joined by a double bond to a single metalloid atom to which at least another group of atoms is attached. 50

24. The process of making an intermediate for use in the preparation of photographic gelatino-silver-halid emulsions, which comprises substantially freeing gelatin from sensitizing compounds and incorporating therein seleno carbamid. 55

25. The process of making an intermediate for use in the preparation of photographic gelatino-silver-halid emulsions, which comprises substantially freeing gelatin from sensitizing compounds, and incorporating therein a sensitizing compound containing a divalent selenium atom directly joined by a double bond to a single metalloid atom to which at least another group of atoms is attached, the amount of said added compound being less than the order of 10 grains for 100 pounds of gelatin (calculated as dry gelatin), and being insufficient to cause immediate fogging tendency 70 in emulsions made from said intermediate.

Signed at Rochester, New York this 18th day of January, 1926.

SAMUEL E. SHEPPARD.